

## UNITED STATES PATENT OFFICE.

JAMES ASTON, OF PITTSBURGH, PENNSYLVANIA, ASSIGNOR TO A. M. BYERS COMPANY, OF PITTSBURGH, PENNSYLVANIA, A CORPORATION OF PENNSYLVANIA.

## MANUFACTURE OF WROUGHT IRON.

No Drawing. Application filed June 8, 1921, Serial No. 476,020. Renewed November 24, 1922.

*To all whom it may concern:*

Be it known that I, JAMES ASTON, a citizen of the United States, residing at Pittsburgh, in the county of Allegheny and State of Pennsylvania, have invented a new and useful Improvement in the Manufacture of Wrought Iron, of which the following is a full, clear, and exact description.

My invention relates to the process of making wrought iron wherein the product of a steel making process is poured into a bath of slag having puddling characteristics to granulate the metal and form a coherent mass of slag and metal, as described in my co-pending applications Serial No. 376,247, filed April 24, 1920, for methods of making wrought iron, and Serial No. 376,388, filed April 24, 1920, for processes of making wrought iron.

In carrying out this process, I have found that as the molten metal is poured into the molten slag the temperature of the slag is raised by the molten metal so that the temperature of the molten slag is liable to rise to or above the melting point of the metal. In case the temperature of the slag bath is allowed to rise, it is liable to reach a range of temperature in which the metal is not properly comminuted or granulated, thus causing imperfect and insufficient slag distribution and even the presence of molten metal, which will injure the product.

I have discovered that this rise into the danger zone of temperature may be avoided either by providing a sufficiently large volume of slag relative to the amount of metal poured in, or by cooling the bath during the introduction of the molten metal, as for instance by feeding in cold pulverized slag or cold comminuted metal. I may use either or both of these ways of preventing the temperature from rising into the danger zone.

The temperature of the product of the steel-making operation may be assumed as being from 2800° to 2900° F. It solidifies at about 2730° F. The slag temperature of an ordinary puddle slag in molten condition is about 2200° to 2300° F. In order to provide for proper welding of the granules in the slag bath to form the mixed coherent mass of slag and metal, a temperature is desired of about 2500° to 2600° F.; but the temperature should not rise beyond the fusion point of the metal, which, as above

stated, is about 2730° F., and is preferably 55 kept well below this latter temperature.

With a fixed quantity of molten slag, as more and more metal is poured into it the equilibrium temperature will rise until, if sufficient metal is poured in, it will reach 60 or pass the melting point of the metal, after which the metal will no longer granulate, but will coalesce into a mass of slagless metal. The higher the initial temperature 65 of the slag, and the higher the temperature of the metal, the sooner this injurious condition will arise.

Taking ordinary average temperatures of metal and a slag of puddling characteristics, I find that to prevent this injurious condition by relative volumes, the volume of slag to metal should be over 1½ to 1, and preferably over 2 to 1. In fact, for complete safety by relative volumes alone, the slag volume may well be increased to 3 volumes 75 of slag to 1 of metal. (Relative weights of 1½ to 1).

But if cold pulverized slag is added to the slag bath during the pouring in of the molten metal, the initial volume of slag 80 relative to metal may, of course be less.

If one volume of slag is used to one volume of metal, cold slag additions should be made to an amount of at least 6% by weight of slag addition relative to the amount of 85 metal poured in, and the cold addition is preferably carried above this percentage to obtain the desired result. For example, with a slag metal ratio of 2 volumes to 1, where the initial temperature of the slag 90 is about 2300° F. and the temperature of the metal about 2900° F., I have added cold pulverized slag in successive small amounts to approximately 12 per cent by weight of metal poured in, with good results.

I have also found that the greater the temperature difference which is maintained between the slag bath and the metal, the more effective is the granulating action. It is, therefore, desirable to keep the temperature difference well away from the danger zone, not only to insure granulating, but to produce efficient thorough granulating.

In any case, the final equilibrium temperature of the bath, after the pouring in of 105 the molten metal is completed, should be below the melting point of the metal; and this may be insured either by a sufficiently

large volume of slag relative to metal, or by cold additions, or by both.

As in my copending applications above referred to, the temperatures, speed of introduction of the metal, amount of cold additions, if used, etc., should be so regulated that the equilibrium of temperature is within the welding range so that the mass of mixed metal and slag will weld together and form a coherent mass as the granules descend through the bath to the lower part of the receptacle or vessel containing the bath. After the operation, the surplus slag may be removed and the mass or ball compressed either in the same receptacle or after removal therefrom.

The advantages of my invention will be obvious to those skilled in the art, since thorough and uniform slag distribution is insured, and large slagless lumps or masses of metal avoided, as is also the presence of molten metal in the bath. For the production of high grade wrought iron, therefore, this invention is highly important, as it insures thorough granulating and very uniform slag distribution. Changes may be made in the particular slag used, although this should be of general puddling characteristics, and in the character of the molten steel product. The bath may be cooled in various ways, and other changes may be made without departing from my invention.

I claim:

1. In the manufacture of wrought iron, the steps consisting of pouring the molten product of a steel-making operation into molten slag, granulating it therein, and maintaining the temperature of the molten slag below the melting point of the metal through said operation.

2. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation.

3. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by artificially cooling the bath.

4. In the manufacture of wrought iron, the steps consisting of subjecting metal to a steel-making operation, pouring the product into molten slag of a lower temperature than the metal to granulate it therein, and keeping the temperature of the molten slag bath

below the melting point of the metal throughout the operation by making cold additions to the bath.

5. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by making additions of cold slag to the bath.

6. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by using a larger volume of slag than the amount of metal poured in.

7. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by using a larger volume of slag than the amount of metal poured in and making cold additions thereto.

8. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by using a volume ratio of at least  $1\frac{1}{2}$  of slag to 1 of metal.

9. In the manufacture of wrought iron, the steps consisting of subjecting metal to a steel-making operation, pouring the product into molten slag of a lower temperature than the metal to granulate it therein, and keeping the temperature of the molten slag bath below the melting point of the metal throughout the operation by using a volume ratio of at least  $1\frac{1}{2}$  of slag to 1 of metal and making cold additions.

10. In the manufacture of wrought iron, the steps consisting of granulating the molten product of the steel-making operation, mixing the granules while retaining at least a part of their original heat with a slag of puddling characteristics, and maintaining the temperature of the molten slag below the melting point of the metal through the mixing operation.

In testimony whereof, I have hereunto set my hand.

JAMES ASTON.